

1,582,347

April 27, 1926.

J. B. READ ET AL.

## SULPHATING PROCESS FOR ORES AND CONCENTRATES

Filed Nov. 26. 1919



J.B. Read and M.F. Coolbaugh. Inventor

३४

Attorney

## UNITED STATES PATENT OFFICE.

JOHN BURNS READ, OF ST. LOUIS, MISSOURI, AND MELVILLE F. COOLBAUGH, OF GOLDEN, COLORADO, ASSIGNEES TO THE COMPLEX ORES RECOVERIES COMPANY, OF DENVER COLORADO, A CORPORATION OF COLORADO.

## SULPHATING PROCESS FOR ORES AND CONCENTRATES.

Application filed November 26, 1919. Serial No. 340,888.

To all whom it may concern:

Be it known that we, JOHN BURNS READ and MELVILLE F. COOLBAUGH, citizens of the United States, residing at St. Louis, Missouri, and Golden, Jefferson County, Colorado, respectively, have invented certain new and useful Improvements in Sulphating Processes for Ores and Concentrates; and we do declare the following to be a full, clear, 10 and exact description of the invention, such as will enable others skilled in the art to which it appertains to make and use the same, reference being had to the accompanying drawings, which form a part of this 15 specification.

This invention relates to a one-step process for treating ores and concentrates to convert them into sulphates, and while it applies particularly to sulphides, and more 20 especially to complex sulphides of lead and zinc, it also applies to oxidized minerals and to mixtures of sulphides and oxidized minerals.

Throughout the present case; the term 25 "ores" is intended to cover not only raw ores but also concentrates, matte, tailings and by-products containing metal or metal compounds in commercial quantities.

The object of this invention is to recover 30 metals from ores. This is accomplished by forming sulphates and separating the soluble sulphates from the insoluble sulphates and other insoluble material by leaching methods.

Heretofore, in attempting to obtain sulphates from sulphides, the efforts have been largely unsuccessful for two reasons; first, because the temperatures could not be properly controlled, since the temperature attained by the combustion of the sulphides, and required for a rapid and complete decomposition of the sulphides, was above the temperature best adapted for the formation 40 of many of the sulphates; and second, because the sulphurous gases and metallic oxide formed by the roast, and the excess of oxygen introduced with the air during roasting were not brought in contact with each other at the proper temperatures to 45 form the desired sulphates, since the gas and ore were traveling in opposite directions.

The present one-step process has four important features: First, the temperature is

controlled by causing the ore or concentrate, and the gaseous products of the roast, to 55 travel in the same direction, that is, "concurrently". By this means the larger portion of the desulphidizing action takes place nearer the feed end of the furnace, and the 60 larger portion of the sulphating action nearer the discharge end of the furnace. The reactions of desulphidizing and sulphating, however, are overlapping. The high temperatures developed by the combustion of the 65 sulphides and required for a rapid and efficient decomposition of the same are maintained in the desulphidizing zone. In this zone only those sulphates will form which have decomposition temperatures higher 70 than the temperature of this zone. The temperature is reduced in the sulphating zone by allowing radiation through the walls of the furnace, or by introducing cold gases directly into the gases of the furnace 75 which are too hot, or by cooling the walls or rabbles of the furnace with cold gases or liquids. In this zone those sulphates continue to form which have decomposition temperatures higher than the temperature 80 of this part of the furnace, and also some unchanged sulphides may be decomposed since the temperature may be sufficiently high for that purpose. Second, much sulphurous gas ( $SO_2$ ) is converted to sulphuric 85 gas ( $SO_3$ ) under the catalytic influence of oxids, chiefly ferric oxid— $Fe_2O_3$ . This action takes place most effectively at temperatures between  $550^{\circ}$  to  $750^{\circ}$  C. Third, these gases and metallic oxids formed by the 90 roast and the oxygen from the excess of air introduced for the roasting are caused by the "concurrent" movement of materials to come into contact with each other at the most efficient temperature for the formation 95 of the desired sulphates. Fourth, a basic ferric sulphate of the type  $Fe_2O_3 \cdot 2SO_3$  is formed from the excess sulphur and iron, which, while insoluble in water, has a positive solvent action in the presence of water 100 on sulphides which have escaped desulphidization and on oxids which have escaped sulphating.

The formation of this basic sulphate takes place between  $425^{\circ}$  and  $650^{\circ}$  C., and is 105 especially effective between  $475^{\circ}$  and  $550^{\circ}$  C.

For the most successful operation of this process, it is necessary to understand the thermal effects which influence the temperatures in each zone of the furnace. In the desulphidizing zone, oxygen unites with the sulphur of the sulphide minerals and forms gases which are principally  $\text{SO}_2$ , and metallic oxids, and liberates a large amount of heat. Oxygen unites also with sulphurous 10 gas ( $\text{SO}_2$ ), forming sulphuric gas ( $\text{SO}_3$ ) under the influence of contact with already oxidized material, notably ferric oxid ( $\text{Fe}_2\text{O}_3$ ). This reaction also liberates heat. The 15 temperature of the mineral particles is considerably higher than the temperature of the gases in this zone, due to the fact that the chemical reaction which liberates the heat takes place in the particles themselves, and also that there is a decided 20 resistance to heat flow from a solid to a gas. In the sulphating zone some heat is evolved by the union of the sulphurous gas and oxygen, and by the union of the sulphuric gas with the metallic oxids. Also in this zone 25 the temperature of the particles is slightly higher than the temperature of the gases. Here, however, the total heat liberated is much less than in the desulphidizing zone not only because the heats of formation of 30 the compounds from their respective constituents are less, but also because not all of the oxids (especially iron) formed in the desulphidizing zone are completely converted to sulphates in the sulphating zone.

35 So long as the materials are properly moved and the temperatures controlled, it is immaterial what the direction of movement is, or what kind of furnace is used. For instance, the furnace may be horizontal, or one 40 slightly inclined from the horizontal either up or down, or a vertical furnace in which ore and gases move down, or a vertical furnace in which the ore, if very fine, is blown up with the gases. In the accompanying 45 drawing, a horizontal furnace of the rotary type, having a slight downward inclination is shown by way of example.

In applying this invention to a complex lead and zinc sulphide, the ore or concentrate, or both, together with air (and fuel if 50 there is not enough sulphide sulphur to give the heat required, and gases containing sulphur if not enough of these would be formed to sulphate the metals desired) are introduced into the head of the furnace. The 55 fuel gases can be separated from the mineral gases can be separated from the mineral 60 charge by the use of a muffle furnace if desirable, although this is not generally necessary. Here most of the desulphidizing is accomplished, and a temperature between 65 600° C. and 1000° C. is generally maintained. The best temperature will depend somewhat upon the particular ore or concentrate treated. In this zone the lead, zinc, iron and copper sulphides are changed prin-

cipally to oxids. Some zinc ferrite may form. Any gold present is changed to or remains as metal, depending upon its original condition, and any silver present is changed to metal or remains as chloride, depending upon its original condition. The sulphur of the sulphides is liberated principally as  $\text{SO}_2$ . But, as stated above,  $\text{SO}_2$  is changed by the catalytic influence of ferric oxid and to a lesser extent by other oxids, into  $\text{SO}_3$ . This 70 gas in turn will act as an oxidizing agent upon undecomposed sulphides with the formation of oxids and  $\text{SO}_2$  again. Since sulphides of iron are readily oxidized by the oxygen of the air forming ferric oxid and sulphurous gas, the ferric oxid becomes quickly available as a catalyst for the formation of sulphuric gas ( $\text{SO}_3$ ). Basic lead sulphate and silver sulphate may form here 75 if the temperatures are not too high.

The converted minerals and gases are 80 gradually moved along together into a cooler intermediate zone, the rate of travel depending upon the time required to decompose the sulphides. In this intermediate zone, 85 sulphides are still decomposing and more sulphates and  $\text{SO}_3$  forming.

After further travel, the converted minerals come to a third zone, wherein the temperature is maintained within limits for the 90 formation of the sulphates desired. Here final traces of sulphides may be decomposed and more  $\text{SO}_3$  formed. For an efficient separation of lead and zinc, a temperature of 95 not less than 380° C. nor more than 850° C. 100 is maintained. In the final discharge from the furnace, the lead will be found as sulphate or basic sulphate; the zinc (including that which in the first zone was converted into zinc ferrite), copper, metallic silver, and 105 silver-chlorids, will be found as sulphates. If the temperature conditions have been properly maintained, the iron will be found as oxid and also as basic ferric sulphate of the type  $\text{Fe}_2\text{O}_3 \cdot 2\text{SO}_3$ , as described below. The 110 metallic gold will be unaffected. But, if the temperature is allowed to drop too low, much normal ferric sulphate will form and interfere with the later recovery of metallic zinc. If the temperature runs too high, zinc 115 sulphate will not form and the zinc and lead compounds can not then be separated. Under no circumstance will any silicic acid 120 form at this place, or in the solution in the subsequent treatment of roasted material 125 with water.

The hot gases in this zone may contain any amount of sulphur gases that will effect sulphating. For instance, the process may be carried on with great efficiency using 125 roaster or other gases containing less than three percent by volume of such sulphur gases, which small amount is that found in many metallurgical gases. When ferric oxid is present in amounts of 2% or greater, 130

when the gases are not passed in excess of the usual roasting rate, and when temperatures are controlled as above stated, almost one hundred percent of the sulphurous and

5 sulphuric gases will be absorbed when they are present in the gas being handled in an amount as low as one percent. When the

10 gases leaving the furnace are high in sulphurous and sulphuric content, portions of

15 these may be returned to the head of the furnace or to the sulphating zone as desired. As indicated above, and as disclosed in the drawings, all the products of combustion, including those from fuel when used, may

20 be carried along through the various zones. These products of combustion from fuels used do not materially affect the process of sulphation, but, as above indicated, a muffle furnace may be employed if advantageous.

25 The products from the third zone are treated with water to dissolve the sulphates of zinc, copper and silver. The solution is filtered from the insoluble residue and the

25 above metals separated from the solution by any suitable method, for instance, electrolysis. The insoluble residue containing the

30 normal or basic lead sulphate or both, the ferric oxide or basic ferric sulphate or both, the metallic gold and any gangue material, can be smelted to recover the values. Any arsenic or antimony impurities in the original ore or concentrate would be either driven off as gas, or left with the residue.

35 We have made the valuable discovery that, during the process of sulphating, if the temperature is controlled within proper limits—380° C. to 600° C. (or even up to 650° C.)—basic ferric sulphate, above men-

40 tioned, is formed from the excess of sulphur and iron which are usually present in complex ores. This basic ferric sulphate is not soluble in water, but in the presence of

45 water it has a very decided solvent action upon sulphides which may have escaped de-

50 sulphidization and upon oxids which may have escaped sulphating. This action causes a change of all convertible oxids and sulphides to sulphates. It is best expressed by the following chemical equations, which probably represent the reactions as related to zinc:



55 Both of these equations show the formation of soluble zinc sulphate which is a desirable product in the separation of lead from zinc in that it insures increased extraction. The basic ferric sulphate here formed is of the type in which the metallic element predomi-

60 In other words, the basic ferric sulphate, altho insoluble in water, enters into the re-

action and is responsible for practically 65 100% conversion of all convertible oxids and sulphides to sulphates, whereby it is possible to obtain nearly complete separation of metals whose sulphates are soluble from those whose sulphates are insoluble. 70

From the foregoing it is seen that the presence of ferric oxide increases the rate and extent of sulphating in two ways: First, by causing the sulphurous gas to become sulphuric gas which is more effective in sulphating and at the same time may act as an oxidizing agent in desulphidizing. Such sulphuric gas is forming in all zones of the furnace though the temperature for the most efficient production of this gas lies between 600° C. and 750° C. Second, by forming basic ferric sulphate from the excess of sulphurous and sulphuric gases, this basic compound in the presence of water still further increasing sulphating. 75

In treating different sulphides from those given in the above illustration, slightly different temperatures may be needed to effect the differential sulphating desired. 85

Naturally occurring oxids, carbonates and 90 like compounds may be mixed with sulphides or sulphur and treated in a similar manner. Also, ferric oxide may be added to oxidized minerals, and sulphurous or sulphuric gases or both added from an independent source. 95 Sulphurous gas may first be passed through or over ferric oxide at a temperature to form sulphuric gas and this passed over the oxidized mineral. In all cases the "concurrent" movement during sulphating is as essential 100 as where desulphidizing precedes sulphating, because of the importance of keeping the mineral particles in contact with the gases for an appreciable length of time, so that chemical reaction can be effected. 105

We claim:

1. A process of sulphating the non-ferrous metal content of sulphide ores, which comprises treating the ores continuously, by continuously advancing the ores, roasting the 110 ores while carrying the temperature of the ores at least as high as the decomposition temperature of copper sulphate to convert the sulphides of the ores principally into oxids, moving the liberated gases in contact with the ores, in the same direction as the ores being treated throughout the process, and subjecting the oxidized material during movement and in the presence of the gases produced in the roasting to a temperature sufficient to form sulphates from the 115 non-ferrous metal content of the ore.

2. A process of sulphating sulphide ores which comprises treating the ore in one step, advancing the ore, roasting the ore in 120 the presence of oxygen at temperatures high enough for the formation of oxids of copper, advancing the liberated gases and the ores.

under treatment in the same direction while in contact with each other, then treating the roasted materials, during agitation and in the presence of said gases at a substantially 5 lower temperature than that used in the roasting operation, to convert the oxids of non-ferrous metals formed in the roasting operation, into sulphates.

3. A process of sulphating ores which comprises roasting sulphide ores containing iron and at least one of the metals copper, lead and zinc, at a temperature of about 600° C. to 1000° C., lowering the temperature of the roasted ore to a temperature at which  $\text{CuSO}_4$  10 is stable, and subjecting the roasted product to the action of oxids of sulphur, and passing the ore and the oxids of sulphur in the same direction through the furnace throughout the entire process.

4. A process of sulphating ores containing iron and sulphatizable metal which comprises feeding such ores to and through a furnace, feeding air to and through such furnace, in the same direction therethrough 20 as the ore, maintaining in the desulphidizing zone a temperature substantially above the temperature of decomposition of at least some of the sulphates of the sulphatizable metals in the ore, whereby the ore is roasted 25 and the metals converted largely into oxids, then lowering the temperature of the roasted material and subjecting the cooled material to the action of gases containing oxids of sulphur, the gases and solids moving in the 30 same direction throughout.

5. A process which comprises first submitting ores containing sulphides in the presence of air, to a relatively high temperature favorable to rapid and efficient desulphidization, carrying the sulphur oxids and the 40 roasted ores together in the same direction into a cooler zone maintained at a temperature favorable to efficient sulphatization of the sulphatizable minerals the movement 45 being concurrent throughout the entire process.

6. A process which consists in submitting ores containing sulphides, including iron sulphide, to a temperature favorable to rapid 50 and efficient roasting and to the conversion of the liberated  $\text{SO}_2$  to  $\text{SO}_3$ , carrying the liberated sulphur oxids together with the roasted ore in the same direction while in the desulphidizing zone and thence into and 55 through a cooler zone in which the temperature is maintained favorable to the efficient sulphatization of the sulphatizable minerals.

7. The herein described process which 60 comprises subjecting an ore containing sulphides and containing commercial quantities of both zinc and lead, to a desulphidizing roast at a temperature at least as high as the decomposition temperature of zinc sulphate, conveying the roasting ore and the gases liberated in the roasting operation to a

cooler zone in which a temperature is maintained below the decomposing temperature of zinc sulphate and subsequently leaching the product, whereby substantially all of the zinc is dissolved and substantially all of the 70 lead is left undissolved.

8. A process of sulphating the non-ferrous metals present in ores containing iron sulphide and zinc or copper compounds, which comprises dead-roasting the iron and copper 75 or zinc content of the ore, cooling the roasted product somewhat, maintaining the roasted ore at a temperature favorable for the formation of  $\text{SO}_3$  from  $\text{SO}_2$  and  $\text{O}_2$ , maintaining the roasted product at a temperature favorable for the formation of anhydrous basic ferric sulphate and maintaining the roasted product at a temperature favorable for the sulphating of the non-ferrous metals, all while passing the ore and the 80 gases in contact with each other in the same direction throughout the entire process.

9. A process of sulphating the non-ferrous metals present in ores containing iron sulphide and zinc or copper compounds, which comprises dead-roasting the iron and copper or zinc content of the ore, cooling the roasted product somewhat, maintaining the roasted ore at a temperature favorable 90 for the formation of  $\text{SO}_3$  from  $\text{SO}_2$  and  $\text{O}_2$ , maintaining the roasted product at a temperature favorable for the formation of anhydrous basic ferric sulphate and maintaining the roasted product at a temperature 95 favorable for the sulphating of the non-ferrous metals, all while passing the ore and the 100 gases in contact with each other in the same direction throughout the entire process.

10. A process which comprises first submitting ores containing sulphur mineral in the presence of air to a relatively high temperature favorable to rapid and efficient liberation of sulphur oxides, carrying the sulphur oxides and the ores along together 110 in the same direction while in the desulphidizing zone, and passing said sulphur oxides and ores into a cooler zone maintained at a temperature favorable to efficient sulphatization of the sulphatizable minerals by said liberated sulphur oxides.

11. A process which comprises submitting ores containing sulphur mineral in the presence of air to a temperature which is at least as high as the decomposition temperature of the sulphates of certain of the non-ferrous sulphatizable metals to produce rapid and efficient liberation of sulphur oxides, carrying the sulphur oxides and the treated ores along together in the same direction while in the desulphidizing zone and 125 passing the same thence into a cooler zone 130

and maintaining said cooler zone at a temperature below said decomposition temperature for the formation of said sulphates of said certain metals.

12. A process which comprises submitting ores containing sulphur mineral in the presence of air to a temperature to roast considerably the greater portion of the sulphides of the ores to oxids and produce rapid and

10 efficient liberation of sulphur oxids with the simultaneous formation of sulphur trioxide, advancing said sulphur oxids including the sulphur trioxide and the roasted ores together into a cooler zone, and maintaining

15 said cooler zone at a temperature favorable to the formation of sulphates of the metals of said ores.

13. A process which comprises submitting ores containing zinc sulphide and iron to

20 a relatively high temperature to produce zinc ferrite and liberate sulphur oxids with the simultaneous formation of sulphur trioxide, continuously moving the minerals and the liberated sulphur oxids including the sulphur trioxide along together into a cooler zone, and maintaining said cooler zone at a temperature favorable to the formation of zinc sulphate from said zinc ferrite and said

30 14. A process which comprises first submitting ores containing sulphur mineral and silver in at least one of the forms of metallic silver, silver chloride and silver sulphide, to a relatively high temperature favorable to

35 rapid and efficient liberation of sulphur oxids and whereby any silver sulphide present is roasted and metallic silver formed, carrying the sulphur oxids and the ores along together and maintaining a temperature favorable to the formation of silver sulphate direct from said metallic silver and silver chloride.

40 15. The process which comprises submitting ores containing zinc sulphides and iron to a relatively high temperature in the presence of air, to produce zinc oxid and iron oxid and sulphur oxids, allowing the temperature to rise sufficiently to produce substantial amounts of zinc ferrite from said zinc oxid and iron oxid, continuously moving the solid material and the gases along together into a cooler zone and maintaining such cooler zone at a temperature favorable to the formation of zinc sulphate from the zinc ferrite and sulphur oxids.

45 16. A process of sulphating ores containing sulphides of iron and of non-ferrous sulphatizable metal capable of forming ferrite, such process comprising roasting the said ores while allowing the temperature in the roasting operation to rise high enough to decompose large amounts of the sulphate of said non-ferrous metal if formed, allowing the formation of ferrite during such operation, progressively moving the ore to

lower temperature zones of the furnace, causing the gases in the furnace to travel through the furnace in the same direction as the ore material, and maintaining in some zone of the furnace a temperature low enough for reaction of the ferrite with the oxids of sulphur.

17. The process of sulphating zinc sulphide or blonde which consists in roasting the material at a temperature of about 900° C., and then subjecting the material to the action of the roast gases at a temperature decreasing from 800° C. to 400° C. and in the presence of iron oxide, while moving said gases in parallel current with the material, all the while passing ore and gases in contact with each other and concurrently throughout the entire process substantially as described.

18. A continuous process of sulphatizing sulphide ore and minerals which comprises roasting the ore in the presence of oxygen at a temperature at least as high as the decomposition temperature of copper sulphate, whereby the minerals are desulphidized efficiently with the formation of oxides, ferrites, sulphates and sulphurous oxide, and with the simultaneous formation of catalyzers for the efficient conversion of sulphurous oxide to sulphuric oxide, all while advancing the ores and gases in the same direction.

19. A one-step continuous process of sulphatizing sulphide ores and minerals which comprises roasting the ore in the presence of oxygen at a temperature at least as high as the decomposition temperature of copper sulphate, whereby the minerals are desulphidized efficiently with the formation of oxides, ferrites, sulphates and sulphurous oxide, and with the simultaneous formation of catalyzers for the efficient conversion of sulphurous oxide to sulphuric oxide, then advancing and gradually cooling the sulphur oxides and roasted ore together and maintaining a temperature favorable to the further formation of sulphates and basic sulphates, all while agitating and advancing the ores and gases in the same direction throughout the entire process, and subsequently leaching the product to separate the soluble sulphates from the insoluble minerals.

20. A process for sulphatizing sulphur bearing minerals containing iron, comprising roasting the minerals at a high temperature in the presence of oxygen while agitating the minerals for the rapid and efficient desulphidization of the minerals with the simultaneous formation of metallic oxides and efficient formation of sulphur trioxide for relatively high concentration of said sulphur trioxide, all while advancing the minerals and liberated gases concurrently, whereby sulphates will form readily at said high temperature.

21. A process for sulphatizing sulphur bearing minerals containing iron, comprising roasting the minerals at a high temperature in the presence of oxygen while agitating the minerals for the rapid and efficient desulphidization of the minerals with the simultaneous formation of metallic oxides and efficient formation of sulphur trioxide for relatively high concentration of said sulphur trioxide, all while advancing the minerals and liberated gases concurrently, whereby sulphates will form readily at said high temperature, and carrying the treated minerals and the gases into a cooler zone maintained at a temperature favorable to the efficient further formation of sulphates of the sulphatizable metals.
22. A method of treating sulphide ores, the step comprising roasting the sulphides at a temperature in excess of 600° C., causing the said ores together with the air required for roasting and the gaseous products of the roast to travel in the same direction through the furnace.
23. In a method of treating sulphide ores, the step comprising causing the said sulphides together with the air required for roasting and the gaseous products of the roast to travel in the same direction through the furnace and at such a temperature as will cause substantial desulphidization of the ore.
24. The method of roasting sulphides to produce sulphate which comprises causing the said sulphides together with the air required for roasting and the gaseous products of the roast to travel in the same direction through the furnace, effecting the desulphidizing action largely near the feed end of the furnace and the sulphating action largely near the discharge end of the furnace.
25. The method of desulphidizing ore containing at least one of the metals, copper and zinc, which comprises roasting the same at a temperature above the decomposition point of the sulphates of at least one of the said metals, causing the said ores together with the air required for roasting and the gaseous products of the roast to travel in the same direction through the furnace.

In testimony whereof we affix our signatures.

JOHN BURNS READ.  
MELVILLE F. COOLBAUGH.